

March 17, 1931.

G. D. CRABBS

1,796,861

PREPARED ROOFING

Filed Sept. 26, 1921



INVENTOR

George D. Crabbs

BY

Geo. W. Miller, Jr.

ATTORNEY

## UNITED STATES PATENT OFFICE

GEORGE D. CRABBS, OF CINCINNATI, OHIO

## PREPARED ROOFING

Application filed September 26, 1921. Serial No. 503,354.

My invention relates to prepared roofing, such as shingles, made with a flexible base saturated with and coated with a bituminous material and surfaced with a layer of mineral particles. By my improvement I have obtained a prepared roofing which is more fire resistant, because it contains an amount of non-inflammable material greatly in excess of 50 per cent, than the prepared roofing 10 heretofore on the market and not only has the advantage of being more fire resistant but also has the advantage of being, when exposed to the weather, less liable to curl.

In the preferred form of my invention 15 shown in the drawing I provide a foundation A of felt or paper composed of a major portion of asbestos fibre, commonly known as XX fibre, and a minor proportion of non-mineral fibre, preferably animal hair, of considerably greater length than the asbestos fibre. In making the foundation I prefer to use approximately 60 per cent XX fibre and 20 40 per cent animal hair. Any fibrous material of a suitable nature could be used in place of the hair but I prefer that it be a fibre of a comparatively stiff nature. These materials are treated and formed into a paper or felt, in the ordinary manner of manufacture of felt. This felt is then saturated with a waterproof 25 saturant, preferably a bituminous saturant such as asphalt after which the felt or paper is coated with a coating B of bituminous material preferably of a softer nature than the saturant and into this coating is embedded 30 any suitable surfacing material C such as slate, crushed asbestos rock, or other mineral granules or particles.

I prefer to use for saturating my roofing, particularly in the manufacture of shingles a 40 saturant of relatively hard asphalt having a penetration not exceeding 11 at 77° F. as determined by the Richardson & Forest penetrometer, while for my coating I use an asphalt which is softer than the saturant. 45 The combination of my fibrous felt with its relatively stiff fibres and the comparatively hard asphalt saturant I have found enables me to make a shingle which has sufficient flexibility and likewise sufficient body to make it 50 substantially non-curling. The employment

for the coating material of an asphalt softer than the asphalt which saturates the mineral felt provides a protective seal, over the foundation, which does not crack when exposed to the sun, as would the harder, saturating asphalt. This results in a considerable prolongation in the life of the roofing material. Where mineral particles are applied to the base, the softer coating also serves to secure them in a place better than would be the case if they were applied to the hard saturating asphalt.

## Claims:

1. In a prepared roofing a flexible foundation, composed of a major proportion of mineral fibre, saturated with a relatively hard asphalt having a penetration not exceeding 11 at 77° F. 65
2. In a prepared roofing a flexible foundation, composed of a major proportion of mineral fibre, saturated with a relatively hard asphalt and coated with a softer asphalt. 70
3. In a prepared roofing a foundation, composed of asbestos fibres in excess of fifty per cent saturated with an asphalt having a penetration point not in excess of 11 and coated with a relatively softer asphalt in which is embedded a layer of mineral. 75
4. In a prepared roofing, a flexible fibrous foundation saturated with a relatively hard asphalt and coated with a softer asphalt. 80
5. In a prepared roofing, a flexible porous fibrous foundation, saturated with a relatively hard asphalt and coated with a softer asphalt. 85
6. In a prepared roofing, a flexible porous non-metallic foundation, saturated with a relatively hard asphalt and coated with a softer asphalt in which is embedded a layer of mineral. 90
7. In a prepared roofing, a flat flexible fibrous foundation, saturated with a relatively hard asphalt and coated with a softer asphalt in which is embedded a layer of mineral. 95
8. In a prepared roofing, a flexible felted porous foundation composed of a major proportion of mineral fiber saturated with a relatively hard asphalt and coated with a softer asphalt. 100

9. In a prepared roofing, a flat flexible porous foundation composed of a major proportion of mineral fiber saturated with a relatively hard asphalt and coated with a 5 softer asphalt.

10. In a prepared roofing, a flat flexible porous foundation composed of a major proportion of mineral fiber saturated with a relatively hard asphalt having a penetration 10 not exceeding 11 at 77° F. and coated with a softer asphalt in which is embedded a layer of mineral.

In testimony whereof, I have signed my name to this specification.

15 **GEORGE D. CRABBS.**

**20****25****30****35****40****45****50****55****60****65**